

3,036,005

HIGH TEMPERATURE LUBRICANT COMPOSITION  
John E. Koch, Jr., Bayonne, N.J., assignor to Celanese Corporation of America, New York, N.Y., a corporation of DelawareNo Drawing. Filed Apr. 23, 1959, Ser. No. 808,325  
17 Claims. (Cl. 252—49.6)

This invention relates to synthetic lubricants and more particularly to ester lubricant compositions which are particularly resistant to high temperature oxidative degradation in the lubrication of jet turbines used in aircraft.

Jet turbines are turbines actuated by the energy of a burning fuel and are used to drive compressors which provide large amounts of air for the burning of the fuel. The combustion of the fuel provides the energy for driving the compressors which serve it with the remainder of the useful energy going into the propulsion of the aircraft. Jet turbine bearings are lubricated by pumping a lubricant to the bearings from a reservoir in a closed system. The design of more powerful jet turbines has led to an increase in the lubricant reservoir temperature and to greater difficulty in maintaining lubricant stability under the more severe conditions. For example, a lubricant which will operate satisfactorily at a reservoir temperature of 250° F. will sludge badly, build up viscosity, develop high acidity and corrode metals at a reservoir temperature of 400° F.

Carboxylic acid esters, such as esters of polyols with alkanoic acids are useful as lubricants and esters of polyols, such as trimethylolpropane, trimethylolethane and pentaerythritol, which have at least two methylol groups bonded to a quaternary carbon atom are particularly useful for good oxidative and thermal stability. However, even these compounds are not stable under oxidative conditions in a system where the reservoir temperature is of the order of 400° F. and the local temperature at the bearings may be as high as 600° to 700° F.

It is an object of this invention to provide a lubricant composition which will withstand oxidative conditions at temperatures of the order of 425° F. and higher for extended periods without substantial degradation.

It is a further object of this invention to provide an additive composition which can enhance the oxidative stability of polyol esters to the desired degree.

The objects of this invention are achieved by providing a high temperature lubricant comprising a major proportion of an alkanoic acid ester of a polyol having at least two methylol groups on a quaternary carbon atom, said alkanoic acid having an average of at least 5 carbon atoms, said ester being stabilized against high temperature oxidative degradation by a minor proportion of a diaromatic secondary amine and a minor proportion of a compound having a phenosilazine ring,



The polyol esters are esterification products of single alkanoic acids, or mixtures of alkanoic acids, with a polyol having at least two, and preferably three, methylol groups on a quaternary carbon atom. Among the polyols which may be used are trimethylolpropane, trimethylolethane, neopentyl glycol, pentaerythritol, 2-butyl-2-ethyl-1,3-propanediol and 2,2,4-trimethyl-1,3-pentanediol.

The alkanoic acids used to make the polyol esters have average chains of at least 5 carbon atoms and preferably from 5 to 8 carbon atoms. The individual acids, where

mixtures are used may range in chain length from 2 to 12 carbon atoms. Normal acids are preferred, although branched alkanoic acids may also be used, particularly those with no more than two carbon atoms in side chain

5 The polyol esters are prepared by the esterification of the polyol in the presence of a slight excess of alkanoic acid, either in the presence or in the absence of an acid catalyst. For optimum heat stability, it is preferred to carry out the reaction in the absence of a catalyst. When a catalyst is used, it is generally used in an amount between about 0.05 and about 1.0 percent, based on the weight of the reactants. The preferred catalysts are toluene sulfonic acid, benzene sulfonic acid, zinc salt, lead salts, and related materials.

10 The esterification temperature is preferably between about 180° and about 240° C. and the reaction period may suitably range from about 6 to about 18 hours. Water is removed by volatilization, preferably in the presence of an azeotroping agent, such as a liquid hydrocarbon.

15 The diaromatic secondary amines include diaryl amine, aryl-alkaryl amines and dialkaryl amines, with the aryl groups preferably having no more than 5 benzene rings and the alkyl substituents, when present, having no more than 24 carbon atoms. Among the specific diaromatic secondary amines which may be used are phenyl  $\alpha$  naphthylamine, p,p' dioctyldiphenylamine and phenyl  $\beta$  naphthylamine.

20 The diaromatic secondary amine is suitably used in amounts between about 0.25 and about 3% by weight based on the polyol ester and most preferably in amounts between about 0.5 and about 2% by weight.

25 The phenosilazine compound, having the structure defined above, preferably has a hydrogen atom or a lower alkyl group bonded to its nitrogen valence and preferably has aromatic rings bonded to its silicon valences.

30 The preferred silicon-containing compound is N-ethyl phenodiphenyl silazine which has the structure:



40

45

50

This compound may be prepared from N-ethyl diphenylamine by first reacting one mol of the latter with two moles of butyl lithium (at 100° C. with a nitrogen purge to sweep out the butane by-product) to produce 2,2-dilithium-N-ethyl diphenylamine and then reacting the last named compound (at 180°—220° C.) with an equimolar proportion of diphenyl dichlorosilane to produce the desired compound.

Another method of preparation involves the reaction of N-ethyl phenothiazine with diphenylsilane in equimolar proportions to produce the desired compound with hydrogen sulfide as a by-product.

60 Other phenosilazine derivatives which may be used include phenodiphenyl silazine, N-methyl-phenodiphenyl silazine, N-isopropyl-phenodiphenyl silazine, N-ethyl phenoditolyl silazine and N-ethyl-phenodinaphthyl silazine, bis-N-ethyl phenosilazine, and bis compounds of the other derivatives mentioned above.

65 The phenosilazine derivative is suitably used in amounts between about 0.25 and about 3% by weight, based on the polyol ester and most preferably in amounts between about 0.5 and about 2% by weight.

It has been found that a combination of the two compounds produces substantially better inhibition of viscosity buildup and of acidity development than either compound alone, even when used in equivalent amounts. trimethylpropane triheptanoate, for example, stabilized with 1% each of N-ethyl-phenodiphenyl silazine and vinyl  $\alpha$ -naphthylamine can withstand 100 hours in a jet turbine engine at a reservoir temperature of 400° F. without excessive viscosity buildup or the development of excessive acidity.

While it is not desired to be bound by any particular theory, it is believed that each of the compounds complements the action of the other to provide the desired protection. It is believed that the phenosilazine derivative functions as an anti-oxidant only at the high temperatures referred to above, and is incapable of retarding oxidation at low and intermediate temperatures. It is

4  
Examples II to VIII

The triheptanoate esters of Examples Ia and Ib were blended with N-ethyl-phenodiphenyl silazine and phenyl  $\alpha$ -naphthylamine in the proportions shown in the table below. The N-ethyl-phenodiphenyl silazine was dissolved, with stirring, after heating the ester to 200° F. and the phenyl  $\alpha$ -naphthylamine was dissolved while cooling the ester back to room temperature. Each blend, in a 100 ml. sample, was heated in a glass tube to the temperature shown in the table while dried air at a rate of 5 l./hr. was blown through the sample. One inch square metal platelets (about 0.032 inch thick) were suspended in the blends and weighed before and after exposure to determine corrosion. Platelets of steel, copper, aluminum, titanium and silver were used except in the case of Example II where only steel was used. The tests were run for 20 hours.

| Example No.                                    | II    | III   | IV    | V     | VI    | VII   | VIII  |
|------------------------------------------------|-------|-------|-------|-------|-------|-------|-------|
| Ester of Example                               | Ia    | Ib    | Ib    | Ib    | Ia    | Ib    | Ia    |
| Percent N-ethyl-phenodiphenyl silazine         | 1.0   | 1.5   | 1.0   | 1.0   | 1.0   | 1.0   | 1.0   |
| Percent Phenyl $\alpha$ -naphthylamine         | 1.0   | 0.5   | 1.0   | 1.0   | 1.0   | 1.0   | 1.0   |
| Temperatures, ° F.                             | 500   | 500   | 500   | 400   | 400   | 450   | 450   |
| Acidity, Mgs. KOH per gm.                      | 9.8   | 12.7  | 7.4   | 0.39  | 0.23  | 3.39  | 2.49  |
| Viscosity, cs. @ 100° F.                       | 22.63 | 21.57 | 21.85 | 16.69 | 16.57 | 17.14 | 18.02 |
| Change in weight of metal specimens, mgs./cm.² | +0.09 | +0.19 | +0.19 | +0.04 | +0.03 | +0.08 | N.C.  |
| Steel                                          |       |       |       |       |       |       |       |
| Copper                                         |       | -0.81 | -0.54 | -0.09 | -0.06 | -0.45 | -0.23 |
| Aluminum                                       |       | +0.12 | +0.14 | +0.05 | +0.07 | +0.03 | -0.01 |
| Titanium                                       |       | +0.11 | +0.09 | +0.06 | +0.03 | +0.02 | N.C.  |
| Silver                                         |       | +0.09 | +0.12 | +0.05 | +0.03 | +0.05 | -0.02 |

so believed that the phenosilazine derivatives are relatively ineffective even at high temperatures once acidity is started to build up. The secondary amine, which itself is incapable of retarding oxidation at high temperatures, serves to retard oxidation and acidity buildup during the warming and cooling periods and permits the phenosilazine derivative to operate at its full effectiveness the higher temperature.

The phenosilazine derivatives and the secondary amines may be advantageously blended together in the desired proportion to produce a combination additive. Or each may be separately dissolved in the polyol ester with the phenosilazine derivative generally being dissolved at a temperature of about 200° F. and the secondary amine at a temperature of about 100-200° F.

Example I

All "parts" in this and succeeding examples are by weight unless otherwise designated.

(a) A reaction mixture was prepared by mixing 1063 parts of heptanoic acid, 350 parts of trimethylolpropane, 50 parts of toluenesulfonic acid and 395 parts of naphtha. The mixture was heated in a reaction still for a total of 1.5 hours with the maximum temperature in the reaction liquid rising to 242° C. At the end of the heating period the naphtha was flashed off. The mixture was then distilled at an absolute pressure of 4-5 mm. Hg and the fraction coming off at a vapor temperature of 255-281° C. is collected. The collected material was given an alkaline wash and a water wash and then dried. The finished methylolpropane triheptanoate had a specific gravity (20/20) of 0.963, an acid number (mg. KOH/g.) of 0.04, hydroxyl content of 0.20 weight percent and a water content of 0.01 weight percent.

(b) Another batch of trimethylolpropane triheptanoate is prepared by a procedure essentially similar to that described above except that the toluenesulfonic acid was omitted in the reaction and that the distillation step was omitted. The product had a specific gravity (20/20) of 0.964, an acid number (mg. KOH/g.) of 0.01 and a water content of 0.01 weight percent.

35 It is to be understood that the foregoing detailed description is merely given by way of illustration and that many variations may be made therein without departing from the spirit of my invention.

Having described my invention, what I desire to secure by Letters Patent is:

40 1. A high temperature lubricant comprising a major proportion of a normally liquid alkanoic acid ester of a polyol having two to four methylol groups on a quaternary carbon atom, said alkanoic acid having an average of at least 5 carbon atoms and the individual acids of which contain 2 to 12 carbon atoms, said ester being stabilized against high temperature oxidative degradation by a minor proportion of a diaromatic secondary amine selected from the group consisting of diaryl amines, aryl alkaryl amines and di-alkaryl amines and a minor proportion of a compound having a phenosilazine ring having its nitrogen valence satisfied by a member of the group consisting of hydrogen and lower alkyl radicals and its silicon valences bonded to aromatic rings.

45 2. A high temperature lubricant comprising a major proportion of a normally liquid alkanoic acid ester of a polyol having three methylol groups on a quaternary carbon atom, said alkanoic acid having an average of at least 5 carbon atoms and the individual acids of which contain 2 to 12 carbon atoms, said ester being stabilized against high temperature oxidative degradation by a minor proportion of a diaromatic secondary amine selected from the group consisting of diaryl amines, aryl alkaryl amines and di-alkaryl amines and a minor proportion of a compound having a phenosilazine ring having its nitrogen valence satisfied by a member of the group consisting of hydrogen and lower alkyl radicals and its silicon valences bonded to aromatic rings.

50 3. A high temperature lubricant comprising a major proportion of an alkanoic acid ester of trimethylolpropane, said alkanoic acid having an average of from 5 to 8 carbon atoms, said ester being stabilized against high temperature oxidative degradation by a minor proportion of a diaromatic secondary amine selected from the group consisting of diaryl amines, aryl alkaryl amines and di-

55 4. A high temperature lubricant comprising a major proportion of a normally liquid alkanoic acid ester of a polyol having two to four methylol groups on a quaternary carbon atom, said alkanoic acid having an average of at least 5 carbon atoms and the individual acids of which contain 2 to 12 carbon atoms, said ester being stabilized against high temperature oxidative degradation by a minor proportion of a diaromatic secondary amine selected from the group consisting of diaryl amines, aryl alkaryl amines and di-

60 5. A high temperature lubricant comprising a major proportion of a normally liquid alkanoic acid ester of a polyol having three methylol groups on a quaternary carbon atom, said alkanoic acid having an average of at least 5 carbon atoms and the individual acids of which contain 2 to 12 carbon atoms, said ester being stabilized against high temperature oxidative degradation by a minor proportion of a diaromatic secondary amine selected from the group consisting of diaryl amines, aryl alkaryl amines and di-

65 6. A high temperature lubricant comprising a major proportion of a normally liquid alkanoic acid ester of a polyol having two to four methylol groups on a quaternary carbon atom, said alkanoic acid having an average of at least 5 carbon atoms and the individual acids of which contain 2 to 12 carbon atoms, said ester being stabilized against high temperature oxidative degradation by a minor proportion of a diaromatic secondary amine selected from the group consisting of diaryl amines, aryl alkaryl amines and di-

70 7. A high temperature lubricant comprising a major proportion of an alkanoic acid ester of trimethylolpropane, said alkanoic acid having an average of from 5 to 8 carbon atoms, said ester being stabilized against high temperature oxidative degradation by a minor proportion of a diaromatic secondary amine selected from the group consisting of diaryl amines, aryl alkaryl amines and di-

alkaryl amines and a minor proportion of a compound having a phenosilazine ring having its nitrogen valence satisfied by a member of the group consisting of hydrogen and lower alkyl radicals and its silicon valences bonded to aromatic rings.

4. A high temperature lubricant comprising a major proportion of trimethylolpropane triheptanoate, said trimethylolpropane triheptanoate being stabilized against high temperature oxidative degradation by a minor proportion of a diaromatic secondary amine selected from the group consisting of diaryl amines, aryl alkaryl amines and di-alkaryl amines and a minor proportion of a compound having a phenosilazine ring having its nitrogen valence satisfied by a member of the group consisting of hydrogen and lower alkyl radicals and its silicon valences bonded to aromatic rings.

5. A high temperature lubricant comprising a major proportion of a normally liquid alkanoic acid ester of a polyol having two to four methylol groups on a quaternary carbon atom, said alkanoic acid having an average of at least 5 carbon atoms and the individual acids of which contain 2 to 12 carbon atoms, said ester being stabilized against high temperature oxidative degradation by a minor proportion of a diaromatic secondary amine selected from the group consisting of diaryl amines, aryl alkaryl amines and di-alkaryl amines and a minor proportion of an N-alkyl-phenodiphenyl silazine.

6. A high temperature lubricant comprising a major proportion of a normally liquid alkanoic acid ester of trimethylolpropane, said alkanoic acid having an average of at least 5 carbon atoms and the individual acids of which contain 2 to 12 carbon atoms, said ester being stabilized against high temperature oxidative degradation by a minor proportion of a diaromatic secondary amine selected from the group consisting of diaryl amines, aryl alkaryl amines and di-alkaryl amines and a minor proportion of an N-alkyl-phenodiphenyl silazine.

7. A high temperature lubricant comprising a major proportion of a normally liquid alkanoic acid ester of a polyol having two to four methylol groups on a quaternary carbon atom, said alkanoic acid having an average of at least 5 carbon atoms and the individual acids of which contain 2 to 12 carbon atoms, said ester being stabilized against high temperature oxidative degradation by a minor proportion of a diaromatic secondary amine selected from the group consisting of diaryl amines, aryl alkaryl amines and di-alkaryl amines and a minor proportion of N-ethyl-phenodiphenyl silazine.

8. A high temperature lubricant comprising a major proportion of an alkanoic acid ester of a polyol having two to four methylol groups on a quaternary carbon atom, said alkanoic acid having an average of from 5 to 8 carbon atoms, said ester being stabilized against high temperature oxidative degradation by a minor proportion of phenyl  $\alpha$ -naphthylamine and a minor proportion of a compound having a phenosilazine ring having its nitrogen valence satisfied by a member of the group consisting of hydrogen and lower alkyl radicals and its silicon valences bonded to aromatic rings.

9. A high temperature lubricant comprising a major proportion of an alkanoic acid ester of a polyol having two to four methylol groups on a quaternary carbon atom, said alkanoic acid having an average of from 5 to 8 carbon atoms, said ester being stabilized against high temperature oxidative degradation by a minor proportion of phenyl  $\alpha$ -naphthylamine and a minor proportion of N-ethyl-phenodiphenyl silazine.

10. A high temperature lubricant comprising a major proportion of an alkanoic acid ester of trimethylolpropane,

said alkanoic acid having an average of from 5 to 8 carbon atoms, said ester being stabilized against high temperature oxidative degradation by from 0.25 to 3 weight percent of phenyl  $\alpha$ -naphthylamine and from 0.25 to 5 weight percent of N-ethyl-phenodiphenyl silazine.

11. The lubricant of claim 1, wherein said diaromatic secondary amine is present in an amount between about 0.25 and 3 weight percent and said phenosilazine compound is present in an amount between about 0.25 and 10 weight percent.

12. A high temperature lubricant comprising a major proportion of trimethylolpropane triheptanoate, said trimethylolpropane triheptanoate being stabilized against high temperature oxidative degradation by from about 0.5 to about 2 weight percent of phenyl  $\alpha$ -naphthylamine and from about 0.5 to about 2 weight percent of N-ethyl-phenodiphenyl silazine.

13. An anti-oxidant composition consisting essentially of a diaromatic secondary amine selected from the group consisting of diaryl amines, aryl alkaryl amines and di-alkaryl amines and a compound having a phenosilazine ring having its nitrogen valence satisfied by a member of the group consisting of hydrogen and lower alkyl radicals and its silicon valences bonded to aromatic rings, said components being present in a weight ratio of 0.25 to 3:0.25.

14. An anti-oxidant composition consisting essentially of a diaromatic secondary amine selected from the group consisting of diaryl amines, aryl alkaryl amines and di-alkaryl amines and a phenosilazine compound having the structure



40 wherein the nitrogen valence is satisfied by a member of the group consisting of hydrogen and lower alkyl radicals and the silicon valences are bonded to aromatic rings, said components being present in a weight ratio of 0.25:3 to 3:0.25.

15. An anti-oxidant composition consisting essentially of phenyl  $\alpha$ -naphthylamine and a compound having a phenosilazine ring having its nitrogen valence satisfied by a member of the group consisting of hydrogen and lower alkyl radicals and its silicon valences bonded to aromatic rings, said components being present in a weight ratio of 0.25:3 to 3:0.25.

16. An anti-oxidant composition consisting essentially of a diaromatic secondary amine and N-ethyl-phenodiphenyl silazine in a weight ratio of 0.25:3 to 3:0.25.

17. An anti-oxidant composition for carboxylic acid lubricants consisting essentially of phenyl  $\alpha$ -naphthylamine and N-ethyl-phenodiphenyl silazine in a weight ratio of 0.25:3 to 3:0.25.

#### References Cited in the file of this patent

#### FOREIGN PATENTS

600,325 Great Britain ----- Apr. 6, 194

#### OTHER REFERENCES

65 Atkins et al.: "Development of Additives and Lubricating Oil Compositions," I. & E. Chem., vol. 39, No. 4, pp. 491-7, April 1947.

Barnes et al.: "Synthetic Ester Lubricants," Lubrication Engineering, pp. 454-8, August 1957.

**Notice of Adverse Decision in Interference**

In Interference No. 93,833 involving Patent No. 3,036,005, J. E. Koch, Jr.,  
HIGH TEMPERATURE LUBRICANT COMPOSITION, final judgment adverse to the patentee was rendered Dec. 20, 1965, as to claims 9, 10,  
12 and 17.  
[Official Gazette June 28, 1966.]